

## UNITED STATES PATENT OFFICE.

MAURICE FOULD, OF PARIS, FRANCE, ASSIGNOR TO SOCIETE ANONYME DES HAUTS FOURNEAUX, FORGES ET ACIERIES DE POMPEY, OF PARIS, FRANCE.

## PROCESS FOR THE MANUFACTURE OF MANGANESE STEELS.

No Drawing.

Application filed July 10, 1923. Serial No. 650,733.

*To all whom it may concern:*

Be it known that I, MAURICE FOULD, citizen of the French Republic, residing at Paris, in the French Republic, have invented new and useful Improvements in Processes for the Manufacture of Manganese Steels, of which the following is a specification.

The present invention has for its object 10 a process for the manufacture in the basic or neutral converter of hard steels containing a large proportion of manganese, such as Hadfield steels for example, by the blowing in said converter of rich spiegels.

15 In a cast iron treated upon a basic lining, the proportion of manganese, after having undergone a great reduction during the period of burning of the silicon, decreases only much more slowly during the decarburation. This is in accordance with the principle stating that carbon, beyond a certain minimum temperature, has a greater affinity for oxygen than any other element. The manganese thus burns in rather 20 great quantity only during the relatively cold period termed sparking period, that is to say before the ignition of the flame of the carbon. As soon as the heating of the whole mass is sufficient to provide for 25 the starting of the decarburation, this latter reaction takes precedence over all the other oxidations which become then only 30 of a minor importance.

With these remarks in view, I had the 35 idea of treating in the basic converter a nonphosphoric cast iron, which, at first sight, would seem unreasonable, but which ensures a very important practical result, as is further set forth, if care is taken to 40 choose as the nonphosphoric cast iron, a high manganese cast iron, containing for example 15 to 20 per cent of manganese, such as high manganese spiegel which always contains the necessary proportion of silicon 45 to ensure the operation which will be further described.

The method of operating is as follows: One brings the liquid spiegel from the blast furnace or any other source (cupola furnace, melting furnace, etc.) into a basic or neutral converter preliminarily heated by preceding operations. The addition of lime is very small or even nil, the slag being made sufficiently basic by the combustion of

the manganese and the wear of the lining. 55 The spiegel normally contains a small amount of silicon whose combustion at the beginning of the blowing operation aids in the increase of temperature necessary to start the decarburation. This heating of the bath is moreover all the more rapid inasmuch as there is not here, as in a normal Thomas operation any cooling action produced by an enormous mass of lime fed into the furnace at the lower outer temperature. 60 65

The operation starts with the combustion of the silicon and then by the combustion of a part of the manganese, and as soon as the temperature is sufficient, the carbon commences to burn; at this time but little silicon remains, but there still remains the major part of the manganese whose elimination will now take place very slowly whereas on the contrary the carbon is rapidly eliminated. The working of the decarburation is examined with the spectroscope by the usual methods, and the operation is stopped when the proportion of carbon is that desired. 70 75

The metal obtained still contains a large proportion of manganese, for example 10 to 12 per cent as for the Hadfield steel whose uses are well known. One can thus, when starting with a suitable cast iron treated by this process, obtain in fact a steel having a predetermined proportion of carbon and manganese. 80 85

Further, after the blowing operation, the treatment of the metal may be completed in the Martin furnace or in an electric furnace, either to change the relative proportions of carbon and manganese within wide limits, or to add new elements, metals or metalloids of a special nature. 90 95

It should be observed that with the general process above described, the quantity of manganese which is oxidized during the starting and which is contained in the slag is not lost; it may be recovered by treating this slag in the blast furnace. 100

Having now described my invention, I declare that what I claim as new and desire to secure by Letters Patent is:

The process for manufacturing high manganese steels which consists in charging into a basic converter a bath of non-phosphoric high manganese cast iron containing more 105

manganese than in the steels to manufacture and less than 5% of carbon and 1% of silicon, in blowing an oxidizing agent through said bath to burn the silicon and 5 a small part of manganese hereby elevating the temperature of the bath to a determined point above which the oxidation of

the carbon supplants that of the manganese, and in continuing to blow said oxidizing agent through the bath hereby decarburizing the latter. <sup>10</sup>

In testimony whereof I have signed my name to this specification.

MAURICE FOULD.